

Patented Aug. 29, 1933

1,924,804

# UNITED STATES PATENT OFFICE

1,924,804

## PROCESS FOR MAKING STAINLESS STEEL

Albert F. Plock, Niagara Falls, N. Y.

No Drawing. Application December 29, 1931  
Serial No. 583,789

2 Claims. (Cl. 75—45)

My invention relates to the manufacture of chromium-steel alloys, particularly the alloys containing chromium or chromium and nickel commonly known as stainless steel or rustless 5 iron.

Chromium alloy steel such as is termed stainless steel has under the prevailing practice been made by the use of low carbon ferro-chromium which is relatively costly to produce and is made 10 use of in a process which is relatively expensive. Such alloy usually contains ten to twenty percent of chromium, sometimes five to twelve percent of nickel, not over .06 to .15 of one percent of carbon, the balance mostly iron. As carbon 15 cannot be reduced after chromium has been introduced into molten iron without loss of chromium, it has been considered necessary that the carbon content in the ferro-chromium introduced into the molten iron be very low.

20 It is the object of my invention to avoid the necessity of using low carbon ferro-chromium and to permit the use of chromium ore by reducing the chromium direct from the ore so as to produce chromium alloy steel and chromium nickel alloy steel at less cost than by the prevailing process.

With this object in view my invention consists in the process hereinafter described and claimed.

In carrying out my process, iron or steel is 30 melted in an electric furnace of usual type to form a bath and is treated with an oxidizing flux of lime and iron ore, or lime and mill scale, for reducing the carbon in the molten bath to about five to ten one-hundredths of one percent depending upon the percentage of carbon desired 35 in the chromium, or chromium-nickel, steel. As soon as the carbon in the molten bath has been reduced to the desired degree the oxidizing slag is raked or poured off and a slag of about four 40 parts of lime to one part fluorspar is added in quantity sufficient to cover the surface of the molten bath to a depth of two or three inches when the slag is treated and the metal of the bath is brought to a good workable temperature.

45 The molten metal of the bath being thus covered with slag of the composition stated, a mixture of chromite, silicon-chromium alloy, lime and fluorspar is slowly charged on top of the layer of slag, that is, charged not faster than 50 the chromium content of the mixture is then being reduced by the silicon in the silicon-chromium alloy.

The silicon-chromium alloy preferred contains 55 fifty-six percent of silicon, twenty-seven percent of chromium, six one-hundredths percent

of carbon and the balance mostly iron. Chromite contains from forty-five to fifty-four percent of chromium oxide  $\text{Cr}_2\text{O}_3$ , and 8 to 15 percent iron. The chromite and the silicon-chromium alloy are both ground fine enough to pass an 8 to 60 60 mesh screen while the lime and fluorspar are left in lumps of about chestnut size. All of the ingredients are intimately mixed.

The percent of silicon and the percent of chromium alloy may be varied from five to ten 65 percent above or below the percentage mentioned.

When slowly charged into the slag as above described the silicon will reduce the chromite, picking up the oxygen and leaving the chromium and 70 iron free to pass into the molten metal below the slag, the silicon being oxidized to silica remaining in the slag.

After the charging of the mixture has been kept up until the desired amount of chromium 75 has been reduced and added to the molten iron about eighty percent of the slag is removed and lime and fluorspar added to form a refining slag and after a short time the alloy is ready to be 80 poured into a ladle to be cast into ingots.

In practical operation in an electric furnace of the common arc type, I have first melted 1100# of steel scrap and reduced the carbon to .06% by means well known to the art. After adding lime and fluorspar to form a slag covering, I 85 have charged a mixture of 500# chromite containing 50%  $\text{Cr}_2\text{O}_3$ , 12%  $\text{FeO}$ , 150# silicon-chromium alloy containing 56% silicon, 27% chromium and 12% iron, 350# burnt lime, and 60# fluorspar, the chromite and silicon-chromium 90 alloy being finely ground and as a result, have produced a fine quality of chromium alloy steel of the following analyses: chromium 15%, silicon .20%, carbon .09%, manganese .29%, at a less cost than by the use of low carbon ferro-chromium as in the general process of making 95 stainless steel. I have also made the so-called 18—8 stainless steel, that is 18% chromium and 8% nickel by adding nickel to the plain low carbon steel bath before the slag covering was 100 added, then following the same procedure as for plain chromium alloy steel. In each case the chromium loss has not exceeded 6% of the amount charged and the carbon held well under 105 .10% in the steel.

Having thus described my invention what I claim is:

1. A process of making an alloy containing iron and chromium which consists in forming a 110 bath of molten iron, reducing its carbon content

by use of an oxidizing flux, removing the oxidizing slag from the surface of the bath, protecting the bath of molten metal by adding lime and fluorspar to form a coating of slag of substantial thickness on the surface of the molten metal, and charging on top of the slag so formed a mixture of chromite and silicon-chromium alloy in pulverized form with lime and fluorspar, the silicon-chromium alloy containing approximately two parts of silicon to one of chromium.

2. A process of making an alloy containing iron and chromium which consists in forming a bath of molten iron, reducing its carbon content

by use of an oxidizing flux, removing the oxidizing slag from the surface of the bath, protecting the bath of molten metal by adding lime and fluorspar to form a coating of slag of substantial thickness on the surface of the molten metal, and charging on top of the slag so formed a mixture of chromite and silicon-chromium alloy in pulverized form with lime and fluorspar, the chromite and silicon-chromium alloy being in the proportions of about fifty parts chromite fifteen parts of silicon chromium alloy.

ALBERT F. PLOCK.

|    |     |
|----|-----|
| 15 | 90  |
| 20 | 95  |
| 25 | 100 |
| 30 | 105 |
| 35 | 110 |
| 40 | 115 |
| 45 | 120 |
| 50 | 125 |
| 55 | 130 |
| 60 | 135 |
| 65 | 140 |
| 70 | 145 |
| 75 | 150 |